

## UNITED STATES PATENT OFFICE

2,604,450

## LUBRICATING GREASE COMPOSITION

Arnold J. Morway, Clark Township, Union County; David W. Young, Roselle, and Delmer L. Cottie, Highland Park, N. J., assignors to Standard Oil Development Company, a corporation of Delaware

No Drawing. Application December 22, 1950.  
Serial No. 202,422

7 Claims. (Cl. 252—42.1)

1

This invention relates to lubricating compositions. Particularly it relates to outstanding synthetic ester base lubricating grease compositions prepared with amounts of soap hitherto thought impossible. More particularly the invention relates to lubricating grease compositions having good light stability, good structural stability and good low temperature properties prepared from a synthetic ester oil and minor amounts of a soap and of an acyl p-amino phenol.

The esters of dibasic carboxylic acids have been found to have properties which make them extremely valuable as synthetic lubricants. Their high boiling points and resulting low vapor pressures at ambient temperatures, their high viscosity indices, their extremely low pour points, and their chemical stability make them of great value in specialized lubrication problems.

It has been known that these synthetic esters may be used for the preparation of lubricating grease compositions. One such grease composition is described in U. S. Patent 2,436,347 issued on February 17, 1948 to J. C. Zimmer and A. J. Morway. The preparation of these synthetic ester base greases, however, is difficult and involves the use of large amounts of soap, in the order of 12-21% by weight. Ordinarily, it is also necessary to use from 0.5-5% of a stabilizer in these synthetic ester base greases, for example an amphoteric metal compound such as an oxide, carbonate, or soap of zinc or aluminum.

It has now been found, and forms the object of this invention, that these desirable synthetic ester base grease compositions may be prepared using relatively minor amounts of the usual grease forming soaps by utilizing the novel oil thickening properties of an N-acyl p-amino phenol having certain specified carbon chain lengths in the aliphatic portion thereof.

The technique of the preparation of these novel lubricating grease compositions is very simple. The synthetic ester lubricant chosen is admixed with from about 1-6% by weight of an alkali metal or alkaline earth metal soap of a high molecular weight substantially saturated fatty acid and heated to a temperature within a range of from 350 to 480° F. with stirring. In a separate kettle from 1.0%-12% by weight of the desired N-acyl p-amino phenol is admixed with a mineral lubricating oil and heated with stirring, to a temperature of approximately 250° F. When the mixture of synthetic ester and soap has cooled to approximately 250° F. the oil-amino phenol mixture is added and the whole mass allowed to cool to room temperature, resulting in a clear solid grease structure.

Among the synthetic ester lubricating oils op-

erable for the preparation of the greases of invention may be any of the aliphatic dibasic acid esters having the general formula:

R'OCRCOOR'

wherein R is a bivalent aliphatic hydrocarbon radical such as methylene, polymethylene, ethylenedene, propylenedene, methyl dimethylene, butylenedene and the like and wherein R' and R'' are branched chain hydrocarbon radicals having from 4 to 22 carbon atoms and may be alike or different. Examples of some of the synthetic esters operable, and covered by the formula above, are the esters of adipic acid, suberic acid, azelaic acid and sebatic acid.

Other synthetic oils which may be used as base stocks for the preparation of very satisfactory grease compositions according to the inventive concept include the polyethers such as the polyglycol ethers and complex esters such as the esters of alkylated succinic acid, "Oxo alcohol" esters of dihydroxy acids, and the like.

The soap constituent of the greases of invention may be any of the alkali metal or alkaline earth metal soaps of the commonly used soap forming acids. Calcium, barium, strontium, sodium or lithium soaps of such materials as hydrogenated fish oil acids, hydrogenated castor oil, stearic acid, hydroxy stearic acid, oleic acid, beef fat, tallow, the saturated or unsaturated glycerides of various fatty acids or mixtures may be used.

The mineral oil used as a dispersant for the amino phenol may be any paraffinic or naphthenic base oil, refined by any of the commonly used refining techniques.

The N-acyl p-amino phenols useful for forming the greases of invention have the following general formula—



wherein R is an alkyl group containing from 16 to 22 carbon atoms, preferably an alkyl group non-benzenoid in nature and wherein R' and R'' are alike or different and are hydrogen atoms or alkyl groups containing from 1 to 20 carbon atoms.

50 The preferred embodiment of this invention contemplates the use of compounds according to the formula above wherein R' and R'' are hydrogen atoms and wherein R is a straight chain aliphatic group containing from 16 to 20 carbon atoms. Exemplary of these preferred compounds are N-palmitoyl p-amino phenol, N-stearoyl p-amino phenol, and N-arachidoyl

Among the synthetic ester lubricating oils op-

p-amino phenol, N-stearoyl p-amino phenol is especially preferred.

The alkylated N-acyl p-amino phenols, exemplified by the formula above where R' and R'' are alkyl groups containing from 1 to 20, preferably 4-15, carbon atoms, are also operable in the instant invention. Compounds such as N-n-valeryl-4-amino-3-pentadecyl phenol, N-n-propanoyl-4-amino-3-pentadecyl phenol, N-n-pentanoyl-4-amino-2,6-di-tert-butyl phenol, N-n-hexoyl-4-amino-2-hexyl phenol are exemplary of these alkylated p-amino phenols.

It is also within the inventive concept to use the N-acyl m-amino phenols, that is those compounds in which the amino group is meta to the hydroxyl group as thickeners.

The preparation of these amino phenols is simply accomplished by admixing the desired acid or acid chloride with the desired p- or m-amino phenol and heating the mixture under proper reaction conditions. The reaction proceeds quite smoothly splitting off water or hydrogen chloride, giving the desired N-acyl p- or m-amino phenol which may then be purified by any of the various methods known to the art. An example of the preparation of one N-acyl p-amino phenol is given below.

One mol of p-amino phenol was placed in a glass round bottomed flask equipped with a reflux condenser with an azeotropic take off side arm. To the flask was then added one mol of stearic acid and 50 grams of xylene. The xylene served as an entraining agent to remove, azeotropically, the water of the reaction. The flask was heated to the xylene refluxing temperature for about five hours, or until such time as the theoretical water (1 mol) was removed. The round bottomed flask was then emptied into an evaporating dish and the mixture heated on a steam bath until the last traces of xylene were removed. The compound was then recrystallized from glacial acetic acid and there resulted colorless N-stearoyl p-amino phenol.

As was mentioned above, the greases of this invention are prepared simply and easily by a blending or mixing operation of two components. One component is a mixture of the chosen synthetic ester and a soap. The synthetic ester may be of any of those listed above and is used in amounts ranging from 34% to 79% by weight, preferably 60-75%. A soap of an alkali metal or an alkaline earth metal and a high molecular weight substantially saturated fatty acid is admixed with the synthetic ester in amounts ranging from 1% to 6%, preferably 3 to 6% by weight. This mixture is heated to a temperature within a range of from 350° to 480° F. with stirring, at which point the heat is removed.

With from 14% to 53% by weight of a refined mineral oil, preferably 15 to 30%, there is admixed, with stirring, from 1.0% to 12%, preferably 1-6%, of the desired N-acyl p-amino phenol. This mixture is then heated to about 250° F. and then blended with the synthetic ester-soap mixture at the same temperature. The total mass is then cooled to room temperature by any of the conventional grease cooling methods and there results a stable translucent grease composition of excellent appearance. (The percentages given above are by weight, based on the weight of the total composition.)

*Example I*

Following the procedure outlined above a lu-

bricating grease composition was prepared according to the following formula—

6.0% lithium stearate  
2.0% stearoyl p-amino phenol  
23.0% refined naphthenic distillate having a viscosity at 210° F. of 35 S. U. S. and a pour point of -45° F.  
69.0% Di-2-ethyl hexyl sebacate

10 Standard inspection tests on the grease of Example I gave the following results—

Dropping point \_\_\_\_\_ °F. 360  
Water solubility (30 min. at 210° F.) \_\_\_\_\_ Nil  
Penetration: (mm./10 at 77° F.) unworked 280  
15 Worked—  
60 strokes ASTM worker \_\_\_\_\_ 310  
80,000 strokes ASTM worker \_\_\_\_\_ 340

*Example II*

20 By the same procedure as in Example I, a grease having the following formula was prepared.

4.0% lithium hydroxy stearate  
2.0% N-palmitoyl p-amino phenol  
25 18.0% refined naphthenic distillate having a viscosity at 210° F. of 35 S. U. S. and a pour point of -45° F.  
76.0% "C<sub>8</sub> Oxo" alcohol ester of sebacic acid.

30 Standard inspection tests upon the grease composition of Example II gave the following results:

Dropping point \_\_\_\_\_ °F. 364  
Water solubility (30 min. at 210° F.) \_\_\_\_\_ Nil  
Penetration: (mm./10 at 77° F.) unworked 310  
35 Worked—  
80 strokes, ASTM worker \_\_\_\_\_ 318  
80,000 strokes, ASTM worker \_\_\_\_\_ 355

To summarize, this invention relates to new and useful lubricating grease compositions and a method of their manufacture having desirable properties of stability, fluctuating temperature lubricating and the like which consists essentially of a synthetic ester thickened to a grease consistency with a minor amount of a soap and from 1.0% to 12% by weight of an N-acyl p-amino phenol having from 16 to 22 carbon atoms in the acyl portion thereof. The greases are prepared by mixing the amino phenol with a small amount of a mineral oil and blending this mixture with the synthetic ester containing dispersed therein a minor amount of an alkali metal or an alkaline earth metal soap of a high molecular weight substantially saturated fatty acid.

55 What is claimed is:

1. A lubricating grease composition comprising from about 34% to 79% by weight of a synthetic ester having the general formula—



60 wherein R is a bivalent hydrocarbon radical of the class consisting of methylene, polymethylene, ethylidene, propylidene, and methyl-dimethylene radicals, and R' and R'' are branched chain hydrocarbon radicals having from 4 to 22 carbon atoms and may be alike or different

65 thickened to a grease consistency with (1) a mineral oil solution of 1 to 12% by weight of a material having the formula—



70 wherein R''' is an aliphatic hydrocarbon radical containing from 16 to 22 carbon atoms

and with (2) from 1% to 6% by weight of a material of the class consisting of alkali metal and alkaline earth metal soaps of high molecular weight substantially saturated fatty acids.

2. A lubricating grease composition consisting essentially of about 34% to 79% of a material having the formula—



wherein R is a bivalent hydrocarbon radical of the class consisting of methylene, polymethylene, ethylidene, propylidene, and methyldimethylene radicals, and R' and R'' are branched chain hydrocarbon radicals, alike or different, containing from 4 to 22 carbon atoms

which has been thickened to a grease consistency with (1) a solution of about 14% to 53% of a mineral oil and about 1% to 12% of an N-acyl p-amino phenol having from 16 to 22 carbon atoms in the acyl portion thereof, and (2) about 1% to 6% of an alkali metal soap of a substantially saturated fatty acid; percentages being by weight, based on the weight of the total composition.

3. A lubricating grease composition consisting essentially of about 64% to 73% of an ester having the general formula—



wherein R' and R'' are branched chain hydrocarbon radicals having from 4 to 22 carbon atoms which has been thickened to a grease consistency with (1) about 3% to 6% of an alkali metal soap of stearic acid and with (2) a solution of about 15% to 30% of a naphthenic mineral oil and about 1 to 6 of an N-acyl p-amino phenol, the acyl group of which contains from 16 to 20 carbon atoms, percentages being by weight, based on the weight of the total composition.

4. A lubricating grease composition according to claim 3 wherein the metal soap is lithium stearate and the p-amino phenol is N-stearoyl p-amino phenol.

5. A lubricating grease composition consisting essentially of about 69% of di-2-ethyl hexyl sebacate thickened to a grease consistency with about 6% of lithium stearate, and a solution of about 2% N-stearoyl p-amino phenol in about 23% of a naphthenic mineral oil, percentages being by weight, based on the weight of the total composition.

6. A process for the preparation of ester base lubricating compositions which comprises the steps of admixing with from 34% to 79% of an ester material having the formula—

## R'OOCR'COOR''

wherein R is a bivalent hydrocarbon radical of the class consisting of methylene, polymethylene, ethylidene, propylidene, and methyldimethylene radicals and R' and R'' are branched chain hydrocarbon radicals, alike or different, containing from 4 to 22 carbon atoms

from 1% to 6% by weight of a metal soap of a high molecular weight substantially saturated fatty acid, heating the mixture while stirring to a temperature within a range of from 350° to 480° F., cooling the mixture to a temperature of about 250° F., blending therewith a mixture of about 14% to 53% of a naphthenic mineral oil and about 1% to 12% of a material having the formula—



wherein R''' is an aliphatic hydrocarbon radical containing from 16 to 20 carbon atoms

said mixture having been heated to a temperature of about 250° F., and cooling the resulting blend to obtain a stable grease composition, percentages given being by weight, based on the weight of the total composition.

7. A process for the preparation of synthetic oil base lubricating grease compositions which comprises the steps of admixing with from 64% to 73% of di-2-ethyl hexyl sebacate, 3 to 6% of lithium stearate, heating the mixture with stirring to about 350° to 480° F., cooling the mixture to a temperature of about 250° F., blending therewith a mixture of about 15% to 30% of a naphthenic, mineral oil containing dissolved therein about 1 to 6% of N-stearoyl p-amino phenol said mixture having been heated to about 250° F., and cooling the resulting blend to obtain a stable grease composition, percentages given being by weight, based on the weight of the total composition.

ARNOLD J. MORWAY.  
DAVID W. YOUNG.  
DELMER L. COTTLE.

## REFERENCES CITED

The following references are of record in the file of this patent:

## UNITED STATES PATENTS

| Number    | Name             | Date          |
|-----------|------------------|---------------|
| 2,436,347 | Zimmer           | Feb. 17, 1948 |
| 2,442,672 | Von Fuchs et al. | June 1, 1948  |
| 2,467,147 | Morway et al.    | Apr. 12, 1949 |